

July 31, 1928.

1,678,825

S. RUBEN

ELECTRIC CURRENT RECTIFIER

Filed March 30, 1927

FIG. 1.



FIG. 2.



INVENTOR.  
Samuel Ruben  
BY  
Mayer, Marples & Watson  
ATTORNEYS.

## UNITED STATES PATENT OFFICE.

SAMUEL RUBEN, OF NEW YORK, N. Y., ASSIGNOR TO RUBEN RECTIFIER CORPORATION, OF ENGLEWOOD, NEW JERSEY, A CORPORATION OF DELAWARE.

ELECTRIC-CURRENT RECTIFIER.

Application filed March 30, 1927. Serial No. 179,479.

This invention relates to electric current rectifiers and the like which employ asymmetric couples of the dry surface-contact variety.

5 Rectifiers of this variety are known which are characterized by the use of a body of relatively electropositive material, employed as one electrode element, disposed in electrical contact with a body of relatively electronegative material employed as the other electrode element; there being an intervening film having inverse current-blocking properties. Such rectifiers depend for their operation upon the resistance and current-blocking characteristics of the film which forms as the result of electrochemical action.

10 Rectifiers depending on these characteristics known to the prior art, have been low in efficiency and limited in their application to 20 small currents, because of improper conditions for film formation and maintenance, and become substantially inoperative after short periods of use.

The invention has for its object generally 25 to provide an improved device of the character described, which is efficient, economical and readily manufactured, and which provides an electronegative electrode element having improved mechanical and electrical characteristics.

30 More specifically, an object is to provide an asymmetric couple which has an electronegative electrode element constructed so as to have both a relatively great mechanical and 35 resistance to compression and a high crystal density.

Other objects of the invention will in part be obvious and will in part appear herein-after.

40 The invention accordingly comprises the features of construction, combinations of elements, and arrangement of parts, which will be exemplified in the constructions hereinafter set forth and the scope of the application of which will be indicated in the 45 claims.

For a fuller understanding of the nature and objects of the invention, reference should be had to the following detailed description taken in connection with the accompanying drawing, in which:

Figure 1 shows diagrammatically a rectifying device constructed in accordance with the present invention; while

55 Fig. 2 is a view showing in cross-section

the electrode elements, indicating symbolically their composition when constructed in accordance with the present invention.

Referring now to the drawing, and particularly to Fig. 2, 10 denotes the electro-positive electrode element which is disposed cooperatively against an electronegative electrode element 11. These elements thus arranged comprise an asymmetric couple and are preferably placed between conducting terminal electrode or end-plates, as shown at 12 in Fig. 1, through which the circuit connections are preferably made. The rectifying device or unit illustrated in Fig. 1 comprises two groups of two couples 70 each, the groups being inverted with respect to each other and disposed adjacent the central electrode plate 13.

The end-plates at the ends of the assembled groups are adapted to be connected in conducting relation by means of a clamping bolt 14, which passes through the couples, but is insulated therefrom, as disclosed in my co-pending application Serial No. 750, 929, filed November 18, 1924. By this arrangement it is seen that the four couples comprise the arms of a Wheatstone bridge, of which the terminals provided at 13 and 14 comprise one diagonal thereof and serve as suitable terminals for the output circuit 80 comprising conductors 15 and 16, leading respectively to the terminals of a direct current-consuming device, here symbolically indicated by the signs + and -. The terminal plates 12, disposed intermediately of the inverted groups, provide the other diagonal 85 of the Wheatstone bridge and serve as suitable terminals for the alternating current input circuit, here shown as comprising the conductors 17 and 18, leading from the low 90 tension side of a suitable step-down transformer 19 here shown as connected to an original source 20 of alternating current; for example, a commercial 60-cycle, 110-volt, A. C. supply.

100 By the arrangement shown, when the conductor 18 has a plus polarity, the electronegative electrode element 11 adjacent thereto will be positively charged and a direct current will pass as the result of rectification from the terminal 14 to the direct current-consuming device; thence by way of the conductor 15 to the central electrode plate 13; and thence by way of a second electronegative electrode element 11 to the terminal 110

plate 12 connected to the conductor 17; and vice versa when the conductor 17 has a plus polarity.

The electropositive electrode element 10 is here a metallic body of substantially any relatively stable but highly active electropositive metal, for example, aluminum, boron, calcium, magnesium or zinc, such as taught in my co-pending application Serial No. 69,215, filed November 16, 1925.

The electronegative electrode element is a metallic compound of a highly electronegative element, which is adapted to form electrochemically an inverse current-blocking film when in contact with the electropositive electrode element. Metallic compounds with elements of the sixth group in the periodic table have this property, particularly maximum valent metallic sulphides, for example, plumbic sulphide, or cupric sulphide. Such sulphides comprise, of course, the basic material which renders operative the electronegative electrode element.

In the practice of the present invention the basic material of the electronegative electrode element is chemically compounded or alloyed with another material, which is adapted to impart a relatively high crystal density and also relatively great mechanical rigidity and strength. The metals of the chromium type or group, namely, chromium, molybdenum and tungsten, have been found to be suitable materials for this purpose. Of these three, chromium is the most practical, since it is readily obtained and introduced in the form of chromium trioxide ( $\text{Cr}_2\text{O}_3$ ).

Metals of the chromium type have a specific resistance materially higher than that possessed by the basic material here employed as a component of the electronegative electrode element. Consequently the adding of such high resistance material results in an increase in the average resistance of the electronegative electrode element, which is desirable, since it insures a proper margin of safety in the resistance factor of the electrode element which is depended upon to provide the energy of film-formation and maintenance out of the  $I^2R$ -losses incident to the passage of current in the electrode element, as set forth in my co-pending applications Serial No. 38,780 filed June 22, 1925, and Serial No. 113,009 filed June 1, 1926, so that there is an adequate supply of the energy necessary for film-formation and maintenance over a relatively wide range of current variation.

Chromium type metals, thus introduced as a component of the electronegative electrode element, may be introduced in varying amounts, depending in a measure upon the range of current variation that the device is intended to operate over. There is, however, an upper limit to the amount which it is not practical to exceed in commercial de-

vices; this limit or maximum being substantially twenty percent (20%) by weight of added chromium type metal in the total mass of the electrode element. This is particularly true for the metal chromium, which, when introduced in the form of chromium trioxide, may be taken in original amounts in a ratio substantially up to three parts of chromium trioxide to seven parts of basic material, as the chromium trioxide suffers reduction when thus combined.

Any suitable method may be adopted for the production of the electronegative electrode element in accordance with the present invention; a preferred method for making cupric-chromium elements, however, involves first a mixing together in proper proportions as above indicated powdered cupric sulphide and powdered chromium trioxide. These ingredients, when properly mixed, are then fused together by the application of heat at a temperature in the neighborhood of 500° C. and cast into suitable forms which may thereafter be machined into the disc-like elements illustrated in the drawing.

The addition of chromium to the electronegative electrode element imparts relatively great mechanical rigidity and strength to the cupric electrode elements, and have in consequence relatively great resistance to mechanical compression. The electronegative electrode elements, when thus constructed, have relatively high internal resistance and high crystal density, and are able to resist compressional stresses up to a maximum in the neighborhood of 150 tons per square inch.

Since certain changes may be made in the above construction and different embodiments of the invention could be made without departing from the scope thereof, it is intended that all matter contained in the above description or shown in the accompanying drawing shall be interpreted as illustrative, and not in a limiting sense.

Having described my invention, what I claim as new and desire to secure by Letters Patent is:

1. In electric current rectifiers and the like, of the dry surface-contact variety, an asymmetric couple having relatively electropositive and electronegative electrode elements adapted for the electrochemical formation and maintenance at their contacting surfaces of an inverse current-blocking film, said electronegative electrode element comprising a metallic compound of an element of the sixth periodic group alloyed with an element of the chromium type.

2. In electric current rectifiers and the like, of the dry surface-contact variety, an asymmetric couple having relatively electropositive and electronegative electrode elements adapted for the electrochemical formation and maintenance at their contacting

- surfaces of an inverse current-blocking film, said electronegative electrode element comprising a metallic sulphide and a compound of chromium, alloyed therewith.
- 5 3. In electric current rectifiers and the like, of the dry surface-contact variety, an asymmetric couple having relatively electro-positive and electronegative electrode elements adapted for the electrochemical formation and maintenance at their contacting surfaces of an inverse current-blocking film, said electronegative electrode element comprising a metallic sulphide and an oxide of chromium taken in an amount adapted to 10 provide a specific resistance in said element sufficient to provide the energy for film formation and maintenance.
4. In electric current rectifiers and the like, of the dry surface-contact variety, an asymmetric couple having relatively electro-positive and electronegative electrode elements adapted for the electrochemical formation and maintenance at their contacting surfaces of an inverse current-blocking film, said electronegative electrode element comprising cupric sulphide and a quantity of an element of the chromium type united chemically so as to impart high density and mechanical rigidity to said element.
- 20 5. In electric current rectifiers and the like, of the dry surface-contact variety, an asymmetric couple having relatively electro-positive and electronegative electrode elements adapted for the electrochemical formation and maintenance at their contacting surfaces of an inverse current-blocking film, said electronegative electrode element comprising a fused mass of cupric sulphide and chromium trioxide, the latter being taken in an amount sufficient to provide the energy for the formation and maintenance of the inverse current-blocking film from the resistance losses incident to the passage of current.
- 25 6. In electric current rectifiers and the like, of the dry surface-contact variety, an asymmetric couple having relatively electro-positive and electronegative electrode elements adapted for the electrochemical formation and maintenance at their contacting surfaces of an inverse current-blocking film, said electronegative electrode element comprising a fused mass of cupric sulphide and chromium trioxide, the latter being taken in an amount sufficient to provide the energy for the formation and maintenance of the inverse current-blocking film from the resistance losses incident to the passage of current.
- 30 7. In electric current rectifiers and the like, of the dry surface-contact variety, an asymmetric couple having relatively electro-positive and electronegative electrode elements adapted for the electrochemical formation and maintenance at their contacting surfaces of an inverse current-blocking film, said electronegative electrode element comprising a fused mass of cupric sulphide and chromium trioxide taken in an amount not to exceed a maximum limit of 20% by weight of chromium in the mass of the electronegative electrode element.
- 35 In testimony whereof I affix my signature.  
SAMUEL RUBEN.